

## UNITED STATES PATENT OFFICE

1,950,116

## METHOD OF CARBONIZING FERROUS METAL

John H. Kyte, Fanwood, N. J., assignor to Swedish Iron & Steel Corporation, New York, N. Y., a corporation of New York

No Drawing. Application November 8, 1932,  
Serial No. 641,740

4 Claims. (Cl. 148—17)

This invention relates to the treatment of ferrous metal and particularly iron for the purpose of increasing its radiation of heat at elevated temperatures.

5 The carbonization of certain metals other than iron has been successfully practiced for some time by heating such metals in hydrocarbon gases at such temperatures as to decompose the hydrocarbon molecule and deposit free carbon upon the 10 surface of the metal. Attempts to carbonize iron and other ferrous metal, however, by similar methods, have heretofore met with great difficulty, due to the failure of the free carbon to uniformly deposit upon the iron and firmly adhere thereto. Certain carbonizing gases which 15 operated satisfactorily in carbonizing nickel, for example, were found to be either entirely inoperative when applied to the carbonization of iron by methods similar to those used in carbonizing 20 nickel, or had the great disadvantage of case hardening the iron to such an extent as to render it unfit for many of the uses for which it was intended.

According to my present invention, ferrous 25 metal is uniformly coated with a firmly adherent carbon deposit and this result may be achieved, if desired, substantially without perceptible case 30 hardening. In principle, the invention involves the preliminary treatment of the ferrous metal under conditions which prepare its surface for the subsequent carbonization at elevated temperature 35 in a carbonizing gas, so that the difficulties heretofore encountered are avoided. This preparation of the surface has been best accomplished by treatment with nitric acid, which appears to be 40 effective by reason of the slight etching of the surface and the formation thereon of a thin oxide film, as a result of which the carbonizing gas is decomposed and carbon set free on the surface of the metal under conditions which ensure uniformity 45 of the coat and firm adherence. The results obtained are consistent with the theory that the oxygen of the oxide film combines with hydrogen of the hydrocarbon gas, setting free carbon at the point of contact. Such surface action, while itself favorable to the adherence of the deposited carbon, is further aided by the irregularities of the etched surface in promoting 50 adherence. The uniformity of the carbon deposit is further consistent with the theory that the oxygen of the oxide film combines with hydrogen of the hydrocarbon gas, in that the formation of the carbon deposit proceeds uniformly over the exposed oxide surface and to a substantially uniform thickness, when the deposition ap-

pears to cease. The invention in its broader aspect is thus not limited to the use of nitric acid in the preliminary treatment of the ferrous metal, but includes treatment with other oxidizing acids or agents which will leave an oxide film on the 60 metal and preferably will have a slight etching action.

I shall describe by way of example the treatment which has been proved satisfactory in carbonizing pure iron sheet. The sheet in the form, for example, of Swedish iron strip is first 65 cleansed thoroughly to free its surface of oil and foreign matter and is then etched in a 15% solution of nitric acid at ordinary temperature for about 1½ minutes time. The time may be varied from say ½ minute to 3 minutes with nitric acid of the strength stated and at the temperature mentioned. Stronger solutions and higher 70 temperatures will naturally require less time, and any of these factors may obviously be varied in 75 accordance with well-known principles. The strip is by this treatment etched and superficially oxidized and thereafter it is thoroughly washed 80 in water to remove any remaining acid. The clean oxidized and etched strip is then run 85 through a carbonizing furnace at a temperature of about 1650° F. This temperature will depend somewhat on the carbonizing gas employed. Such gas may be straight illuminating gas or mixtures thereof with other hydrocarbon 90 containing gases, but the invention in its broad sense is not limited to a particular carbonizing gas and others may be substituted for those mentioned. With any of these gases the temperature may be 95 varied within wide limits, such as for example from 1400° F. to 1800° F., although better results are obtained between 1500° F. and 1750° F., and in practice I prefer to keep within about 50° of 1650° F. temperature, where illuminating gas is employed and a good black deposit is required. 100

The time required to obtain a satisfactory deposit will vary somewhat with the temperature and the character of the carbonizing gas. Where the strip is fed continuously through a carbonizing furnace of standard design, the speed 105 of the strip may readily be regulated by observation of the result, to secure and maintain the desired quality of deposit. For carbonizing already formed sheet, such as for example the plates of thermionic tubes, five or six minutes exposure to the carbonizing gas at the temperatures mentioned will ordinarily give satisfactory results, but here again the observation of the result is the best guide to the proper regulation of 110

the time and temperature with respect to each particular carbonizing gas.

Carbonized strip obtained by the method described may be stamped and formed into finished shapes with little or no loss of carbon from the surface, with the result that the finished object will retain satisfactory heat radiating properties, whether carbonized before or after forming.

With regard to the case hardening effect which has represented a serious difficulty in previous attempts to carbonize iron, it is found that little or no difficulty will be encountered from this cause when carbonizing from straight illuminating gas or other mixtures in which constituents are present such as the hydrogen and carbon monoxide of the illuminating gas to reduce the concentration of the decomposable hydrocarbon. It is also to be noted that the case hardening effect involves a time element which is dependent upon the composition of the carbonizing gas, and in the practice of my invention, under the principles explained, case hardening may readily be avoided as the deposition of the carbon is completed before case hardening has had time to develop to any appreciable extent.

As previously explained, the broad principles of the invention are not limited to the use of specific materials or reagents, and these may ac-

cordingly be varied by the substitution of well-known equivalents. I have found, however, that the preliminary treatment with nitric acid as the etching and oxidizing agent, and the carbonizing with illuminating gas give particularly favorable results on pure iron, and hence the use of these is claimed as a preferred embodiment of the invention.

I claim:—

1. Method of carbonizing ferrous metal which comprises acting upon the surface with nitric acid and later exposing it to carbonizing gas at carbonizing temperature. 85

2. Method of carbonizing iron which comprises treating the surface with nitric acid, and thereafter subjecting it to carbonization temperature in a gas containing carbonizable and non-carbonizable constituents. 90

3. Method of carbonizing iron which comprises treating the surface with nitric acid, and thereafter subjecting it to carbonization temperature in illuminating gas. 95

4. Method of carbonizing substantially pure iron which comprises etching and oxidizing the surface with nitric acid and carbonizing it in the presence of illuminating gas at about 1600° F. to 1700° F. 100

JOHN H. KYTE.

30

105

35

110

40

115

45

120

50

125

55

130

60

135

65

140

70

145

75

150